

W. JENKINS,  
STAY BOLT IRON,  
APPLICATION FILED DEC. 23, 1916.

1,231,898.

Patented July 3, 1917



WITNESS:

Arthur Symmentrett

INVENTOR  
Weslon Jenkins  
BY  
Symmentrett Bradley Lechner Fowles  
ATTORNEY

# UNITED STATES PATENT OFFICE.

WESTON JENKINS, OF ROME, NEW YORK, ASSIGNOR TO ROME MERCHANT IRON MILL,  
OF ROME, NEW YORK, A CORPORATION OF NEW YORK.

## STAY-BOLT IRON.

1,231,898.

Specification of Letters Patent.

Patented July 3, 1917.

Original application filed June 29, 1916, Serial No. 106,578. Divided and this application filed December 23, 1916. Serial No. 138,583.

*To all whom it may concern:*

Be it known that I, WESTON JENKINS, a citizen of the United States, residing at Rome, county of Oneida, and State of New York, have invented certain new and useful Improvements in Stay-Bolt Irons, of which the following is a specification.

This invention relates in general to a tubular bar, as a new article of manufacture, and it has particular reference to a stay-bolt iron as a new article of manufacture. This is a division of my co-pending application, Serial Number 106,578, filed June 29, 1916. One of the primary objects of my invention consists in producing, as a new article of manufacture, an improved hollow rod or similar article, such for example as a stay-bolt, the same being constructed in such manner as to secure maximum strength with no wastage of metal while at the same time the contour of the exterior surface and of the opening is maintained uniform and true. Another of the objects of my invention resides in the provision of an improved construction of hollow rods, such as stay-bolts, whereby a superior product and a uniformity in product are obtained. One of the more specific objects of my invention resides in the provision, as a new article of manufacture, of a hollow stay-bolt iron which is composed of a plurality of complementary or counterpart sections which are placed together to form the stay-bolt, and welded by uniform inward radial pressure.

The foregoing, together with such other objects as may hereinafter appear, or are incident to my invention, I obtain by means of a construction, the preferred embodiment of which I have shown in the accompanying drawings as applied to stay-bolts. Of the drawings—

Figure 1 is an isometric projection of the preferred form of section of wrought iron used in making articles according to my invention; Fig. 2 is a cross-sectional view through three sections such as shown in Fig. 1 after they have been brought together but before they have been welded; Fig. 3 is a cross-sectional view through a completed piece of stay-bolt iron as formed by my invention, the lines marking the divisions being such as would appear when a completed iron

is etched with a suitable etching chemical; Fig. 4 is a plan view more or less conventionalized and on a greatly reduced scale of a furnace and draw-bench suggesting a convenient arrangement of apparatus for producing articles made according to my invention; Fig. 5 is a front face view of a bell-shaped die such as is preferably used in connection therewith; Fig. 6 is a cross-sectional view through the die shown in Fig. 5; Fig. 7 is an isometric projection of a draw-head that may be conveniently utilized to hold the dies; Fig. 8 is a cross-sectional view through a group of three sections of wrought iron of modified form after they have been brought together but before being welded; Fig. 9 is a cross-sectional view through three sections of another modified form that may be used in practising my invention, the pieces being shown after they have been brought together but before being welded; Figs. 10 and 11 are isometric projections of two sections of wrought iron shaped to carry out my invention in its simplest form; Fig. 12 is a cross-sectional view of the parts shown in Figs. 10 and 11 after they have been placed together but before being welded; Fig. 13 indicates the application of my invention to the construction of a form which is square both inside and outside.

My invention will be described as applied to the production of stay-bolts. On account of the peculiar strain placed upon stay-bolts, under service conditions, it is practically universally required that they be formed of wrought iron having certain characteristics and that they be provided with a small central opening in order to give warning by steam or water whenever a stay-bolt has been broken or strained so as to be fractured part way through.

My invention consists in a hollow stay-bolt of wrought iron which is composed of wrought iron sections, more or less sector-shaped in cross-section, with their vertex portions cut away to form the central opening; such sections being welded together to form a hollow cylinder, by uniform inward radial pressure, obtained preferably by drawing the bundle of sections through a die. The stay-bolt, thus produced, is, as an article, superior to standard stay-bolts, not

only in the strength and disposition of the fibers of metal, and consequently in the strength of the bolt as a whole, but also in the contour, not only of the exterior but also of the interior of the bolt, the symmetry of which is maintained with a far greater degree of perfection.

The nature of my invention and the advantages thereof will be better understood by the following statement of one of the methods by means of which my new article of manufacture is produced.

The first step in practising my invention is to form the weldable metal of the proper quality, such for example as wrought iron, into sections of the desired length which shall be of such shape in cross-section as to be sector-shaped or some part of a circle and preferably an aliquot part of a circle. Thus, in Figs. 1 and 2 there are shown such sections 15, each of which is substantially a third of a circle in cross-section, but it will be obvious that other sector-shaped sections may be used such as a quadrant-shaped piece or pieces 20 which have a more acute angle between their plain sides than ninety degrees. I prefer, however, to use sections such as section 16 and particularly such a section provided with interlocking means such as shown in 25 Fig. 9, for reasons hereinafter stated.

The sections of wrought iron furthermore have their vertex portions cut away or grooved as plainly shown in the drawings. Such grooves 17 preferably being so formed 30 as to have a center common with the center of the sector of said sections. A convenient way to form the sections of wrought iron into proper sector-like shape with their re-entering grooves 17 is by rolling the iron to 35 that shape, but other means may be used if convenient.

I then bring together the proper number of sector-like sections to form therefrom a hollow cylinder of which the walls are relatively thick and the central opening 18 formed from the various grooves 17 is relatively small.

The group or "pile" 19 of sections is then heated by any suitable means such as in a furnace 20 until said group or pile has been brought throughout its length to a proper welding heat. Then the pile or group of sections is passed through a bell-shaped die or dies whereby the different sections are 50 welded together into a solid uniform mass but with the central opening 18 still maintained through the mass which is now a piece of hollow stay-bolt iron.

As suggestive means for performing these operations by machinery I have shown the furnace 20 of any suitable form or character to produce the desired heat and of a length sufficient to contain the piles. Preferably also the furnace will be of such width 55 and so constructed as to receive thereinto a

number of piles 19 of these sections side by side in order to carry on the process as efficiently as possible. Closely located outside the furnace 20 is the draw-head 21 with its slot 22 in which is placed a die or a number of dies 23. The die has a circular opening 24 therein of tapering or bell-shaped form as plainly shown in Fig. 6. The die is placed in the slot 22 of the draw-head with its side 25 which has the smaller end of the aperture 24 against the shoulder 26 in the draw-head beyond which is the smaller slot 27 of a size a little larger than the smallest diameter of the aperture 24 in the die.

As the end of the pile 19 of sections properly raised to welded heat comes from the furnace it is led through the bell-shaped die 23 in the draw-head 21 and the rest of the pile 19 drawn through said die by means of the power-operated chain 28 upon the draw-bench 29. Any desired means may be used for introducing the end of the heated sections through the die and connecting them to the drawing chain 28.

As the pile 19 or bundle of sections so heated are thus drawn through the die 23 the adjacent sides of contiguous sections are pressed closely together and are welded together without closing up the small central opening 18. As the bundles of sections are closely circular in outline and as the aperture of the die is circular and of slightly less diameter than the pile 19 of sections presented thereto, it will be apparent that the whole mass is subjected to equal pressure inwardly from all directions toward the center. The result of this equal inward compression all around the circle of the pile being welded together with the drawing action is to reduce the cross-sectional area 100 of the pile and at the same time lengthen the iron being operated upon. The effect of this peculiar uniform inward pressure, as produced for example by drawing the pile through a die, will be best understood by 105 comparing a pile before being operated on with the finished product, reference being had particularly to Figs. 2 and 3.

For this specific example I shall assume that the pile (Fig. 2) has an outside diameter of 1.5" and an inside diameter of .45", leaving the thickness of the wall .525". For a pile having these dimensions I prefer to use dies so constructed that, for a given quality of wrought iron or other weldable metal, and for given heat conditions, when the desired number of passes have been made, a finished hollow bar will be produced having an outside diameter of 1" with an inside diameter of .25", thus leaving the thickness of the wall .375". It will be observed by comparing these dimensions that the inside diameter bears substantially the same proportion to the outside diameter of the finished product as does the internal di- 130

diameter of the pile, before being operated on, to its outside diameter. It will be seen, therefore, that while the external diameter of the pile is considerably reduced during the operation, because of the fact that the variance in the proportion between the internal diameters is very slight, the pile is drawn out and lengthened without the presence of injurious upsetting or distorting action on the metal, the amount of upset being practically negligible. Stated in other words, the uniform inward pressure on the sections compresses and elongates rather than upsets and distorts the metal acted upon, which obviously produces a finished product the characteristics of which are enhanced rather than injured. It will thus be seen that the different sections are welded into one homogeneous mass, the fibers of the wrought iron being compressed and forced together and drawn out so as to bring out the full life, nature or ductility of the wrought metal again after it has been heated. The finished product has therefore maximum inherent strength characteristics, is perfect in external symmetry, and the small internal opening is maintained without distortion. It will also be noted that a minimum amount of metal is required and that the finished product is less expensive than similar articles in which the central opening is drilled.

I have found that stay-bolts for example of this construction are far superior to stay-bolts produced by the well-known methods at present employed in this art.

Where I employ sections which are so formed that the relation between the sections is somewhat in the nature of an arch, I secure additional advantages. Thus, taking the construction shown in Fig. 2, in which the pile is composed of three sections, it will be observed that the pressure on the sections, as shown by the large arrows, results in components, as indicated by the small arrows, which directly increase the welding effect on the sections. To be specific, pressure applied at the juncture of two sections is directly resolved into welding components on the two faces of the third section; and pressure, for example, exerted at the middle of a section resolves itself into two welding components on the remaining two sections, which obviously results in thoroughly welding the sections into a homogeneous finished product, especially where the operations are carried out in such manner as to substantially eliminate upsetting or distorting of the metal during the drawing operation, as previously pointed out.

It will be understood of course that my invention is not restricted to the use of piles or to the production of finished rods having the exact dimensions or proportions heretofore given. By modifying, for example the

shape of the dies, the heat treatment, or the character of the metal, I can produce a finished product having, within certain limits, any desired relation to the original pile or any desired proportionate distribution of metal. To illustrate, I can produce from piles of the same dimensions, finished rods in which the size of the central opening may vary within certain limits and still maintain its external and internal symmetry without injurious upsetting or distortion of the metal.

In the drawings I have illustrated the sections so far described as being truly-sector-shaped in cross-section and substantially this form is preferred because it results in a more uniform distribution of the pressure and a more uniform welding of the iron. It will be obvious, however, that the exterior surfaces may deviate quite a little from true sector shape and still be within the claims of my invention; for instance, irregularity in the arc of the sector or upon the plain surfaces thereof may be present and still obtain a satisfactory result. In fact, in Fig. 8, I have shown a modification of the form of the sections so as to have sections 31 with angular faces 32 which are not exactly radii of the arc surface of the section but are arranged at a slightly smaller angle to each other than in a true sector. This results in the sections 31 when brought together meeting toward the central opening 18, but being slightly separated from each other at the outer surface of the cylinder. This formation has some advantages, in that the first welding is effected toward the central opening and by the time the crevices between the outer surfaces of the sections have been welded it is certain that the weld has been made all the way through to the central opening.

In Fig. 9 I have shown a further and preferred construction of sections, in that the sections 16 here shown have one of their angularly arranged sides provided with a projection or ridge 34 and the other angular face provided with a similar shaped depression or groove 35. It will be obvious that when the proper number of sections of this character are brought together they will fit together or interlock to a certain extent, in that the ridges 34 will engage or fit into the depressions 35. This results in a larger surface to weld and in providing for an easier weld by reason of the interfitting of parts which furthermore maintains the parts in alignment until completely welded. Such arrangement also facilitates the handling of the groups of sections preliminary to the welding steps.

I prefer to form the sections to be used so as to be equal and aliquot parts of the circle. In this way for any given size of stay-bolt iron only one form or size of sec-

tion need be provided. Furthermore, by having the parts equal, whether two, three, four or more parts be used to make the pile or bundle of sections, they will fit together 5 in the same way and the inward compression as from the dies will distribute that pressure equally among the different sections and so obtain an evenness of welding and an evenness of compression of the material that 10 would not be obtained were some of the sections smaller than others.

The term "sector" or "sector-like," as found in this specification, is used in its broad sense.

15 I claim:

1. As a new article of manufacture, a tubular bar comprising a plurality of sector-like sections adapted to be welded together by uniform inward pressure, the vertices of

the sections being cut away to form a central opening.

2. As a new article of manufacture, a hollow stay-bolt comprised of three complementary wrought iron sections grooved to form a central opening when the sections 25 are brought together, said sections being welded together by uniform inward radial pressure.

3. As a new article of manufacture, a hollow bar comprised of a plurality of weldable 30 metal sections each having a portion cut away to provide a central opening when the sections are brought together, said sections adapted to be welded together by uniform inward pressure.

In testimony whereof I have hereunto signed my name.

WESTON JENKINS.